

No. 755,215.

PATENTED MAR. 22, 1904.

W. B. BURROW.  
CONVERTER FOR MAKING STEEL, &c.  
APPLICATION FILED MAY 17, 1892.

APPLICATION FILED MAY 17, 1902.

NO MODEL,

2 SHEETS—SHEET 1.



Witnesses  
J. S. Hall  
A. B. Teller.

Walter B. Burrow, Inventor

No. 755,215.

PATENTED MAR. 22, 1904.

W. B. BURROW.

CONVERTER FOR MAKING STEEL, &c.

APPLICATION FILED MAY 17, 1902.

NO MODEL.

2 SHEETS—SHEET 2.



Witnesses

J. S. Hall

A. B. Feldner

Walter B. Burrow, Inventor

## UNITED STATES PATENT OFFICE.

WALTER B. BURROW, OF NORFOLK, VIRGINIA.

## CONVERTER FOR MAKING STEEL, &amp;c.

SPECIFICATION forming part of Letters Patent No. 755,215, dated March 22, 1904.

Application filed May 17, 1902. Serial No. 107,814. (No model.)

*To all whom it may concern:*

Be it known that I, WALTER B. BURROW, a citizen of the United States, residing at Norfolk, in the county of Norfolk and State of Virginia, have invented a new and useful Converter for Making Steel and Similar Material, of which the following is a specification.

My invention relates to converters for making malleable iron and steel from molten cast-iron and for purifying the same.

The converter differs from those ordinarily in use, as it is operated in an inclined position or horizontally, according to circumstances, and in this way a larger area and volume of metal is more uniformly treated than is possible in other converters. The converter assumes different angles during its operation, all of which do not approach the perpendicular unless the converter is revolved on its axis at the conclusion of the process, as will be herein-after described.

Referring to the drawings, in which like characters of reference indicate similar parts in all the views, Figure 1 is a sectional elevation through the converter shell, lining, corrugations or ribs, and wind-box. In this view the converter-bottom is lower than its outlet or nose. Fig. 2 is a cross-section on the line 1 2 in Fig. 1. Fig. 3 is a part elevation of the converter and wind-box, showing the blast-pipes and regulating-valves. Fig. 4 is a sectional elevation in perspective of the wind-box, showing the divisions or compartments and the deflecting-plates. Fig. 5 is a view of a part of one of the corrugations or ribs looking from the bottom of the converter toward its outlet.

In the drawings, A is the converter-shell. B is the refractory lining. C is the converter-bottom or closed end. D is the converter-bottom plate. E is the slag-door lining. F is the slag-door frame. G represents the vertical or fining twyters which extend through the lining and the corrugations or ribs I. The twyters G blow parallel with the bottom C of the converter and toward the plain lining B and are spaced in suitable rows around the concavity of the corrugations or ribs and extend to the axis or

a little below, as shown in Fig. 2. The lower ends of the twyters connect with divisions in the wind-box J, from which the twyters are supplied with the blast.

H represents the horizontal or dephosphorizing twyters and are located in the corrugations or ribs; but their outlets are below the twyters G and are at right angles to them. The shape of the twyters is that of an inverted L, as shown in Fig. 1. The last row of the twyters H discharges against the bottom C of the converter, and those toward the outlet or nose of the vessel impinge upon the basic material of the ribs on their backs or plain sides, so that the metal is constantly thrown upon the purifying material of which they are constructed. The lower ends of the twyters are connected to different compartments of the wind-box J from those supplying the twyters G. The twyters H are suitably spaced, as shown in Fig. 2.

I represents the refractory ribs or corrugations located above and forming a part of the lining B and are placed on the pouring side of the converter or on its back, if the direction of the discharge of the converter is considered as its front when it is in a vertical position. The twyters G and H are formed in the ribs or corrugations and spaced on the face and sides, respectively, and the shape of the openings made by ramming the material around a pattern, which is afterward withdrawn.

The wind-box J is located on the pouring side or back of the converter and is divided into as many compartments or boxes as there are ribs or corrugations I. The wind-box is also provided with angle or deflecting plates, their object being to guide pulverulent purifying material into the twyters G and H as may be required. As shown in Fig. 1, each upper compartment supplies two rows of twyters; but any combination can be made as desired. The wind-box J is provided with doors L and blast-inlet pipes M.

K is the main blast-feed pipe supplied by the pipe P from the axis or trunnions T.

R represents the valves for regulating the blast-pressure and for cutting off the blast when the twyters are clear of the metal and

the converter is turned completely over or in a vertical position.

When the converter is inclined, as indicated in Fig. 1, the metal-level assumes an angle, as shown at 5, the metal being thinnest over the extreme front twy whole G and thickest over the ones near the bottom C. In this manner the blast acts unevenly and the degree of decarbonization can be varied by tilting the converter and uncovering one or more corrugations or ribs. By treating different thickness of metal variations can be made in the quality of the product and ranging from a mild casting to a superior Bessemer steel.

15 In using pulverulent purifying material I operate the converter when it is horizontal or at an angle, as shown in Fig. 1, until the period known as the "after blow" approaches, at which point I lower the converter in the direction of the arrow 4 until the metal covers the bottom C and the angle 5 is greater. The finely-divided purifying material is then blown into the metal by the twy whole H in such quantity as to saturate the phosphorus or other impurities in the bath. In addition the metal is violently dashed against the blank sides of the ribs or corrugations and by the erosion of the basic ribs causes an intimate contact and to mix with the iron or steel. 25 30 The finished product is poured into molds by tilting the converter in the direction of the arrow 3 or the converter turned over and poured from the plain side. The molten slag is withdrawn as it accumulates by the door E, and the converter is tilted until the metal line or level is even with the opening and the slag run out. The rest of the operation is conducted in the ordinary manner, and known rules of the art of pneumatic steel manufacture can be applied to my invention unless where otherwise specified.

Besides giving many varieties of steel the metallic bath is exposed to a large area of basic material, and a pure product is the result.

45 Having described my invention, what I claim, and desire to secure by Letters Patent, is—

1. A horizontally - operated centrally - pivoted converter for making malleable iron and 50 steel having vertical and horizontal twy whole in the direction of the length of the converter, the said converter or vessel revolving completely through different angles on its axis or trunnions as described.

2. A horizontally-operated tilting converter 55 for making iron and steel, having a plurality of refractory ribs, corrugations or bands, integral with and extending above the lining of the converter; to or near the axis or trunnions, the said ribs or corrugations suitably spaced in the direction of the length of the vessel and occupying one-half of the inner circumference of the converter, and the said ribs or bands containing horizontal and vertical twy whole or blast-orifices, the said twy whole discharging at right angles to each other, as described.

3. A horizontally - operated converter for molten iron and steel having a plurality of twy whole spaced along its length and refractory 70 corrugations or ribs on the inner circumference of the lining and the vertical and horizontal twy whole through the said corrugations or ribs to the wind-box, the horizontal twy whole having their direction of discharge at right 75 angles to the vertical twy whole and blowing toward the closed end of the converter, the said twy whole supplied by the blast from a wind-box on the pouring side of the vessel as described.

4. A horizontally - operated pivoted converter having vertical and horizontal twy whole spaced along the length of the converter and having their direction of discharge at right angles to each other and refractory corrugations or ribs projecting above the lining, to 85 and above the axis of the converter and a horizontally-divided wind box or reservoir having inclined guide and deflecting plates, and regulating valves and pipes, controlling the blast in each division of the said wind-box, as described.

5. A horizontally - operated movable converter for making steel having vertical and horizontal twy whole having their direction of discharge at right angles to each other, and 95 refractory ribs or corrugations carrying the said twy whole, and a horizontally-divided wind-box having deflecting-plates, nozzles, blast-pipes, regulating-valves and a slag-door at the bottom or closed end of the converter, as 100 described.

In testimony whereof I affix my signature in presence of two witnesses.

WALTER B: BURROW.

Witnesses:

J. M. NEWBURN,  
JOHN L. FLETCHER.